

Aug. 30, 1966

5 W. K. WARNOCK ET AL  
PROCESS OF MANUFACTURING PRESS-FREE GARMENT  
WITH RETAINED CREESES  
Filed April 8, 1963

3,268,915

WITH RETAINED CREASES  
Filed April 8, 1963

Fig. 1.



Fig. 2.



Fig. 4.



Fig. 5.

INVENTORS  
WILLIAM K. WARNOCK  
FRANK G. HUBENER  
BY  
*Arington L. White*  
ATTORNEY

1

3,268,915

## PROCESS OF MANUFACTURING PRESS-FREE GARMENT WITH RETAINED CREASES

William K. Warnock, Kentfield, and Frank G. Hubener, San Carlos, Calif., assignors, by mesne assignments, to Koraftron Company, Inc., San Francisco, Calif., a corporation of California

Filed Apr. 8, 1963, Ser. No. 271,107

7 Claims. (Cl. 2—243)

The invention, in general, relates to improvements in outerwear. More particularly, the invention relates to the production of washable garments which withstand repeated washing and which are neat and ready-to-wear without pressing.

While our present invention is directed generally to our disclosures in our existing Letters Patent, No. 2,974-432, issued March 14, 1961, and entitled "Press-Free Crease Retained Garments and Method of Manufacture Thereof," it is principally directed to improvements of the inventions therein described and claimed, as will more particularly appear hereinafter.

A primary object of our present invention is to provide improved washable garments which are unrestricted as to style, size, design and type and which are ready-to-wear after repeated washings without pressing.

Another important object of the invention is to provide an improved process of manufacturing washable press-free garments of the indicated nature which is additionally characterized by affording garments with creases retained therein after repeated washings.

A still further object of our invention is to provide improved washable garments and an improved process of manufacture thereof which affords the utilization of chemically treated fabrics which have been retained on the shelf for an appreciable period without cutting for garment making.

Another object of the present invention is to provide improved garments and an improved process of the indicated nature wherein chemicals impregnated into the garment fabrics are retained uncured for an appreciable period of time without decomposition.

A still further object of our invention is to provide improved washable garments of the indicated nature from chemically treated fabrics wherein the chemical used is maintained in uncured stable equilibrium for longer periods without deterioration and without loss of effectiveness until final curing upon completion of manufacture of the garments at which time they are rendered water-insoluble.

Other objects of the invention, together with some of the advantageous features thereof, will appear from the following description of a preferred embodiment of the invention which is illustrated in the accompanying drawings. It is to be understood, however, that we are not to be limited to the precise embodiment shown nor to the precise order of steps of the process described, as our invention, as defined in the appended claims, can be embodied in a plurality and variety of forms and can be practiced in a plurality and variety of ways.

In its preferred form, our product invention preferably comprises washable press-free garments of any style, size, design or type with creases retained therein and containing a polymerized resinous compound which is water-insoluble and which contains means for maintaining the texture and tensile strength of the fabrics from which the garments are made over an appreciable period and despite repeated washings of the garments.

A preferred mode of manufacturing our aforesaid washable press-free garments, with retained creases therein after repeated washings, comprises the steps of impregnating a fabric with an aqueous solution of a compound

2

containing a thermosetting substance as its major constituent and a fabric conditioner, and a catalyst for extending the duration whereunder the said substance is retained in the fabric in an unset state in the absence of a setting temperature, and a wetting agent for aiding the penetration and saturation of the fabric with said compound, thereafter removing excess solution from the fabric to an extent as to retain approximately 85% to 100% of said thermosetting substance in the fabric, drying the fabric at a temperature below that for setting said substance and to an extent that a moisture content of approximately 8% to 10% is retained therein, thereafter cutting the fabric containing the substance in an unset state to the size, shape, style and type of a desired garment, sewing the garment fabric to provide desired seams, finishing the garment to desired style and design, then imparting at least one crease in the finished garment at a selected area thereof consistent with the style and design of the desired garment under pressure and at a temperature to pre-set said substance at said area, and finally curing or setting the contained substance in situ to a water-insoluble state so that the completed garment is press-free and retains the imparted crease after repeated washing thereof.

Referring to the drawings:

FIG. 1 is a sectional elevational view of one type of oven that can be employed as a component of our improved process, this view illustrating in full lines a treated completed garment suspended from a rack mounted on a portable track.

FIG. 2 is a side elevational view of a preferred embodiment of a garment, as exemplified in a pair of trousers, treated in accordance with our preferred mode of manufacturing the garment.

FIG. 3 a fragmentary front perspective view of a heat and pressure element which constitutes another component of our preferred mode of manufacturing our improved washable press-free garments with sharp creases retained therein after repeated washings.

FIG. 4 is an enlarged fragmentary detail of our preferred embodiment of the invention in a treated garment, this view showing the preferred type of seam employed therein.

FIG. 5 is a cross-sectional view taken on the line 5—5 of FIG. 2.

We have illustrated schematically in the annexed drawings certain equipment which is presently being used after the completion of the manufacture of garments from chemically treated fabric in accordance with our improvements hereinafter more particularly described. However, it is to be understood that any other suitable equipment devised for the same purposes as that shown and for accomplishing the objects herein stated can be substituted for the equipment illustrated. For example, it is entirely feasible and it is contemplated by us to suspend the completed garment from a conveyor which will carry a succession of the garments into and through an oven maintained at a suitable temperature for curing the chemicals contained in the garments to a water-insoluble state. Moreover, the equipment illustrated in FIG. 3 for conditioning the contained chemicals for final setting or curing during their oven treatment likewise can be altered to any other heat and pressure applicator capable of effecting such pre-setting of the chemicals under controlled conditions.

While our improvements are entirely suitable and adaptable for impregnating cellulosic fabrics including blends thereof with man made materials, such as 100% cotton fabrics, viscose rayon and similar blends, we shall describe our present invention, for the sake of brevity and simplicity only, in the environment of fabrics of the latter nature, i.e., cottons and rayons and variations or

combinations thereof. And, of course, the improvements extend to the impregnation of cotton stretch fabrics that result from the slack mercerization process wherein the fabrics are allowed to shrink without restrictive tension in a 25% to 30% solution of caustic soda at approximately 30° C.; the extent of conversion from unmercerized to mercerized being related to the amount of unrestricted shrinkage and the temperature of the washing water although both shrinkage and crystalline conversion become constant after one minute of immersion in the caustic solution. Further, that while any one of a number of different thermosetting chemicals can be employed for preparing the fabric-impregnating solution containing the specified components, we shall describe our present improvements for brevity and simplicity, in the field of thermosetting resins as we have had excellent results with such substances in combination with the components hereinafter delineated in producing our improved washable press-free garments with retained sharp creases therein after repeated washings. As to the cotton stretch fabrics, there is substantially complete recovery and complete shape retention in all press-free washable garments manufactured in accordance with our present improvements with no evidence of bagginess at knee or elbow areas after an appreciable number of washings.

As illustrated in FIG. 1, we provide as our end product, a washable garment 11 containing a cured chemical compound 12 which has been rendered water-insoluble; the cured chemical compound forming a constituent of the fabric of which the garment is made so as to afford a garment that is press-free with retained creases 13 and 14 therein after repeated washings. Thus, the garments are ready-to-wear upon the drying thereof after each washing without having to resort to pressing the garment before donning the same. The garment 11 is completely manufactured from fabric containing the chemical compound 12 in an unset or uncured condition and after completion, including imparting creases therein at desired areas, the garment 11, as well as others similarly processed and completed, may conveniently be disposed on a rack 16, using a standard garment hanger 17 for each garment; the rack 16 being securely mounted on a mobile truck 18, or the like, for movement into and out of a garment-setting oven 19.

In accordance with our present improvements, we preferably utilize unfinished fabrics and if finished each fabric should initially be thoroughly washed in a suitable aqueous soap solution containing a detergent so as to remove starch, gelatin, glucose, dextrose, coloring matter and other impurities, thus avoiding undue stiffening of the fabric during processing. The thus washed fabric should then be rinsed thoroughly in clear water. The unfinished fabric, or thoroughly washed finished fabric is then conveniently wound on rolls for subsequent padding operations.

Each selected fabric from which garments are to be made is unwound slowly from a roll thereof and passed through a conventional dipping or padding machine, not shown, to be thoroughly impregnated with an aqueous solution of a water-soluble thermosetting compound. Preferably, the fabrics are double-dipped in the above mentioned aqueous solution in order to insure approximately 85%–100% pick-up of the solution by the fabrics, and we preferably pre-agitate the solution constantly before each dipping operation as well as maintain the temperature of the solution between approximately 120° F. to 130° F. In this padding step, the fabric containing the thermosetting chemical preferably is passed through rollers for removing excess solutions but, the rollers are so controlled that approximately 85% to 100% by weight of the solution is retained in the fabric.

Thereafter, the impregnated fabric is conveyed onto a standard tenter frame, also not shown, and simultaneously partially dried as it passes along the frame, and is finally wound onto a suitable roller for convenient handling and

rewinding in convenient lengths on other rollers for storage or for transportation to a garment cutting room. In accordance with our invention, the drying temperature to which the fabric is subjected while passing along the tenter frame is maintained between approximately 200° F. and 220° F., which is below the temperature at which the impregnated compound will set or be cured. That is to say, the drying temperature is well below the curing temperature of the chemical solution introduced into the fabric. We so control the drying of the fabric by maintaining the temperature in the range stated as well as by moving the fabric along the tenter frame at a speed of approximately 10 to 15 yards per minute, that the extent of the drying is such that approximately 8% to 10% of moisture is retained therein. All of the foregoing steps are substantially the same as heretofore disclosed in our above mentioned Letters Patent, with the exception of the composition of the aqueous solution, as hereinafter delineated.

In order to stabilize the uncured chemical compound in situ, as introduced into each fabric, for an appreciable period of time before the fabric is cut and sewn into a garment, we preferably include in the aqueous solution of thermosetting compound, a catalyst possessing the property of retarding activation of the chemical solution to any appreciable extent. With this retarding catalyst in the compound, it is possible to process voluminous quantities of a number of fabrics long prior to the making up of garments therefrom, and to keep the processed fabrics on shelves in storage for appreciable periods of time, in some instances for six months, without affecting the final curing or setting of the compounds to a water insoluble state. We also include in our preferred embodiment, in addition to the catalyst mentioned, ingredients having the properties of fortifying or reinforcing the fabric so that its tendency to tear and abrade is materially reduced and its tendency to lose its tensile strength is appreciably reduced. A suitable wetting agent for aiding the dispersion of the aqueous solution of thermosetting compound throughout the fabric also preferably is made a part of our improved compound.

Whenever it is desired to manufacture garments in any style, size, type or design from any fabric processed as hereinabove set forth, the requisite amount of yardage of the fabric is removed from storage, and delivered to a garment cutting room. The fabric is cut, sewn and finished in the garment cutting room and is transferred to a space containing suitable pressing equipment for imparting creases in the completed garments at locations therein consistent with the style and design of each garment, and at the same time presetting the aqueous thermosetting solution contained in the garment at the areas of the imparted creases. Whenever the terms presetting or pre-set are used herein, we mean that the chemicals contained in the fabrics of which the garments are made are subjected to heat and pressure of such degree that these chemicals are substantially cured or set to a water-insoluble state. In our improved processes, this pre-setting occurs at the areas of imparted creases to afford durable, sharp-creases after repeated garment washings as well as at the seams to insure non-puckering. Thus, the creases and seams are pre-set. We have diagrammatically illustrated in FIG. 3 of the annexed drawings, as an example of pressing equipment, a conventional so-called hot head for pressing creases 13 and 14 in the slacks or trousers 11 shown in FIG. 2; such pressing equipment being either pneumatically or hydraulically operated and including a pedestal 21 for elevating the parts to be used to a desired level for an operator, a padded lower element or buck 22 supported on the top of the pedestal and adapted to receive the legs of pants to be pressed, together with a shaped and polished heated head 23 which is pivotally mounted on the pedestal at the rear thereof and adapted to be swung into close proximity and overlying relation to the top of the padded

buck 22 thereby to apply pressure and heat to the pant legs at the proper area for pressing sharp creases in the legs of the garment 11 at desired locations.

The operator, of course, must align the pant legs properly on the front half and the rear half of the buck 22, such as placing the outside leg of one pair of pants 11 on the front half of the buck 22 and the inside leg of another pair of pants on the rear half of the padded buck. In this manner, two garments are handled on each pressing operation. The swing of the heated head 23 into engagement with the pant legs is effected either by manually throwing a switch or by pedal movement of the switch to open the pneumatic or hydraulic valve controlled lines leading thereto, all not shown. The application of the heated head 23, which is supplied with steam from a source, not shown, to the desired garment area on the padded buck 22 for a predetermined time in order to effect sharp creases at the requisite locations. In the case of pants, the head 23 is usually applied to the pant legs for a period ranging between 15 seconds to 30 seconds per leg to impart the sharp creases 13 and 14 therein. When the foot pedal is released, or the manual switch is thrown in the opposite direction as the case may be, the head 23 opens and returns to its initial position. The garment is then removed from the hot head and one garment is re-laid to impart a crease to its other leg and the operator also lays another garment on the buck 22 to apply a crease to its other leg, and the pressing steps repeated. The heated head 23 need not be a so-called double leg finishing press as it is entirely feasible to practice our process using pressing equipment in which but one garment is laid on the buck first in one position and then another for creasing the two legs of a pair of trousers separately. Other pressing units can be utilized for other garments for pressing garment edges, cuffs, collars and the like.

While our improved washable press-free garments can be manufactured with different types of seam construction, we have had most effective results and preferably construct the garments with underpressed open seams with the seam edges, as indicated at 26 and 27 in FIG. 4 of the annexed drawings, lying flat to the garment. As is customary, the seams should be opened and under-pressed with a hot dry iron to be followed by top pressing either on a conventional buck press or by a hot head, as depicted in FIG. 3. We have found that the presetting of the aqueous solution contained in the completed garments at the locations of imparted creases and of the flat seams not only results in the provision and retention of sharp creases in the garments despite repeated washings thereof but also the seams remain smooth and flat with no puckering thereof. This has been found especially true when the final curing and setting in situ of the garment-contained thermosetting compound is not effected in the garment-setting oven 19 for an appreciable time after the imparted creases have been pre-set by the hot head.

At any time after the garments have been completed by cutting, sewing, finishing and pressing, preferably using a hot head for pre-setting creases and seams, as aforesaid, which may include pleating by a mechanical pleating step, each entire garment 11, impregnated with the initially water-soluble thermosetting compound hereinabove mentioned and hereinafter delineated, and having portions of such impregnated compound pre-set adjacent areas of the imparted creases 13 and 14 and at the edges 26 and 27 of the side seams of the garment, is disposed along with other garments similarly processed into the garment-setting oven 19 to effect the setting of the compound in situ thus to cure the contained compound and render the same water-insoluble. Any suitable oven 19 can be employed as long as it is provided with suitable controls for regulating the temperature within the oven and, if gas fired, for regulating by means of suitable throttles, the air and gas flow to maintain the temperature between predetermined low and high values. The oven 19 pre-

ferably should be provided with suitable vents, not shown, to permit escape of air as well as of vapors resulting from the curing or setting of the garment-contained thermosetting compound. Also suitable thermo-couples, not shown, may be suspended within the oven at various locations for testing temperature conditions and for indicating the necessity for throttling the air and gas flow to bring the oven temperature to desired levels. It is to be appreciated that different temperatures are required to cure the thermosetting compounds in different garments, such variations in setting temperatures being dependent in part upon the nature and texture of the fabric of which the garment is made and in which the chemical is contained. The range of temperature in the oven for lighter garments can be from 300° F. to 325° F. and when heavier garments are cured therein the temperature should be elevated to 350° F., with a setting time in all cases ranging between 10 minutes to 20 minutes.

While we have illustrated an oven in FIG. 1 wherein the garments are disposed for a predetermined period of time and exposed to the elevated temperatures indicated, it is entirely feasible to effect the final setting of the contained thermosetting compound by conveying the garments in succession through a specially constructed oven having an open passageway therethrough, all not shown, with the same effective result of curing the compound to a water-insoluble state. Any suitable conveyor for the garments can be employed, such as an overhead monorail from which the individual garments 11 can be pivotally suspended to effect a slow rotation of each garment as it is being moved slowly along the monorail through the passageway of such suggested oven. The particular construction of such open passage-way oven will be described and claimed in a subsequent application.

Our preferred aqueous solution of a thermosetting compound can be altered to some extent for processing different fabrics, the essence of our concept as described and claimed in our above mentioned Letters Patent being that the solution remains unset or uncured until after the completion of the garment. The present invention not only resides in the presetting of the uncured solution in certain areas of the garment, such as at the location of creases, seams, edges and the like, to insure the retention of sharp creases and non-puckered seams or edges after repeated washings, but also resides in an improved formulation of the aqueous solution of thermosetting compound for holding the solution in stable equilibrium within the garment without being activated or without its deterioration or loss of effectiveness and capacity to be cured and set to a water-insoluble state despite the lapse of appreciable periods of time between the time of impregnation of the fabric with the initially water-soluble solution and the time of manufacture and completion of garments from such chemically treated fabrics. To this end, we have formulated our improved compounds as set out in the following examples for impregnation into the indicated fabrics:

*Example I.—100% cotton fabrics*

|                                                                               |         |    |
|-------------------------------------------------------------------------------|---------|----|
| Urea formaldehyde resin, 50% concentrate with approximately 50% water         | gallons | 6  |
| Fabric conditioner, stearamide with dispersion of melamine formaldehyde resin | lbs.    | 16 |
| Catalyst, magnesium chloride hexahydrate                                      |         |    |
| $MgCl_2 \cdot 6H_2O$                                                          | lbs.    | 7½ |
| Wetting agent                                                                 | quart   | 1  |
| Water, to bring to                                                            | gallons | 50 |

The foregoing aqueous solution can be prepared in any desired quantity for dipping of 100% cotton fabric therein to thoroughly impregnate the fabric with the solution. While any water-soluble resin can constitute a major constituent of the aqueous solution, we have had excellent results with an aqueous solution of a urea formaldehyde resin presently available on the market under the trademark "Resloom E-50" and comprising approximately 50% urea formaldehyde resin and approx-

imately 50% water. Any one of a number of fabric conditioners that are water-soluble can form a constituent of the aqueous solution, in the proportionate amount thereof indicated in the above Example I, and we have had consistently good results in the employment of a product presently being marketed under the trademark "Aerotex Permel B" and comprising an equal solids mix of methylol, stearamide and methylated trimethylol melamine. As we have stated above, a significant departure of our present compound from the thermosetting compound delineated in our above mentioned Letters Patent resides in the catalyst employed in our improved thermosetting compound. In our present improvement, we have included a catalyst which will maintain the compound substantially in stable equilibrium in the fabric for a period that appreciably lengthens the shelf-life of the treated fabric. Such catalyst is generally available on the market, and preferably comprises an inorganic, water-soluble metallic salt. The improved compound of our present invention contains as a catalyst magnesium chloride hexahydrate ( $MgCl_2 \cdot 6H_2O$ ). As an agent to assist the dispersion of the aqueous solution uniformly throughout the fabric, and penetration thereof, any suitable wetting agent may be employed, such as that presently available on the market under the trademark "Nekal WS-21" comprising an aqueous solution of a sulfonated aliphatic polyester commonly known in the art as an anionic surfactant. Any suitable finisher to firm up the fabric, such as a water soluble gum or the like, may be added to the solution in minor quantity, if desired. Such a gum can be presently purchased on the market under the trademark "Penford Gum."

Garments manufactured from pure 100% cotton impregnated with the aqueous solution of Example I and processed in accordance with the above delineated steps with the compound retained unset and in stable equilibrium until the garments have been completely manufactured and thereafter set and cured to a water-insoluble state, have withstood approximately 30 washings and yet retained sharp creases without requiring pressing before donning and wear.

*Example II.—100% cotton fabrics*

Urea formaldehyde resin, 50% concentrate with approximately 50% water \_\_\_\_\_ gallons 6  
 Fabric conditioner—stearamide with dispersion of melamine formaldehyde resin in the proportion of 33% by weight of stearamide and 67% by weight of resin \_\_\_\_\_ lbs 16  
 Catalyst, magnesium chloride hexahydrate  $MgCl_2 \cdot 6H_2O$  \_\_\_\_\_ lbs 7½  
 Polyethylene emulsion \_\_\_\_\_ lbs 12  
 Wetting agent \_\_\_\_\_ quart 1  
 Water, to bring solution to \_\_\_\_\_ gallons 50

In the formulation of Example II, the polyethylene emulsion comprising polyethylene stabilized with a small amount of a dispersing agent was found effective in strengthening the treated fabric against tearing and improving abrasion resistance of the fabric, and therefore useful in the manufacturing of garments from carded cotton or the like. The remaining components of the aqueous solution need not be altered for manufacturing our washable press-free garments with retained sharp creases therein.

*Example III.—100% viscose rayon*

Urea formaldehyde resin, 50% concentrate with 50% water \_\_\_\_\_ gallons 12  
 Fabric conditioner, stearamide with dispersion of melamine formaldehyde resin in the proportion by weight of 33% stearamide and 67% resin \_\_\_\_\_ lbs 16  
 Catalyst, magnesium chloride hexahydrate  $MgCl_2 \cdot 6H_2O$  \_\_\_\_\_ lbs 15  
 Elvanol, 72-60 fabric conditioner \_\_\_\_\_ lbs 2  
 Wetting agent \_\_\_\_\_ quart 1  
 Water, to bring to \_\_\_\_\_ gallons 50

In our improved water soluble thermosetting compound for rayon fabrics, we preferably use the additional fabric conditioner presently available on the market under the tradename "Elvanol #72-60," and comprising polyvinyl alcohol, and increase the proportions, per 50 gallons of water, of both the urea formaldehyde resin and the stearamide with melamine formaldehyde resin dispersion, for the most effective results in impregnating the rayon and following out the remaining steps of the process as above outlined.

Other formulations of our improved chemical compound for impregnating other textile yardage, whether entirely cotton, or composed partly of cotton and partly of rayon or blends thereof with man made materials, can comprise any one of the following:

*Example IV*

|                                                         |         |    |
|---------------------------------------------------------|---------|----|
| Urea formaldehyde resin, 50% concentrate with 50% water | gallons | 6  |
| Stearamide, with melamine formaldehyde                  | lbs     | 8  |
| Magnesium chloride hexahydrate, $MgCl_2 \cdot 6H_2O$    | lbs     | 7½ |
| Fabric conditioner ("Synolube Pe")                      | lbs     | 12 |
| Wetting agent                                           | quart   | 1  |
| Water, to bring to                                      | gallons | 50 |

*Example V*

|                                                           |         |    |
|-----------------------------------------------------------|---------|----|
| Urea formaldehyde resin, 50% concentrate with 50% water   | gallons | 9  |
| Stearamide with dispersion of melamine formaldehyde resin | lbs     | 18 |
| Magnesium chloride hexahydrate $MgCl_2 \cdot 6H_2O$       | lbs     | 10 |
| Fabric conditioner (Polyethylene emulsion)                | lbs     | 12 |
| Wetting agent                                             | quart   | 1  |
| Water, to bring to                                        | gallons | 50 |

It is to be understood that any one of the formulations set out in Examples I-V, inclusive, may be varied within slight proportions without departing from the scope and effectiveness thereof; it being kept in mind that the catalyst should not be changed since it serves the important object of retarding or delaying the activation or curing of the compound in the fabric until subjected to a temperature sufficiently high to effect setting thereof to a water-insoluble state or, in other words, of maintaining the compound in an unset state of stable equilibrium in the fabrics for extended periods of time and until after the garments have been completed.

We would also like it to be understood that the important factor of pre-setting the compound in certain crease areas of the finished garment and at seams should be followed in order to obtain effective results with sharp creases and unpuckered seams after repeated washings.

The appended claims are to be accorded a range of equivalents commensurate in scope with the advance made over the prior art.

Wherever the term "wetting agent" is used in the specification and claims, we mean any one of a group of sulfonated aliphatic polyesters which is soluble in water in all proportions and which is known in the art as an anionic surfactant.

We claim:

1. A process of manufacturing garments of any style, size, design and type which are press-free with sharp imparted creases retained therein after repeated washings; said process comprising the steps of impregnating fabrics with an aqueous solution of a thermosetting compound containing a catalyst possessing the property of maintaining the compound in stable equilibrium in the fabrics for appreciable periods at temperatures below the setting temperature of the compound, drying the fabrics containing said compound at a temperature below setting temperature of said compound and to an extent that approximately 8% to 10% of moisture is retained therein, thereafter cutting said fabrics containing said compound

while in an unset state to the size, shape and design of desired garments, sewing the fabrics to provide garment seams located at the areas to be creased, finishing the cut and sewn fabrics to completed garments of desired styles and designs, thereafter imparting at least one crease in said completed garment consistent with the desired style and design of the garments, and at the same time pre-setting said garment containing compound at the locations of said seams and said crease, and finally curing the impregnated partially dried and partially pre-set completed garments to water-insolubilize the contained compound in situ so that the completed garments are press-free with a retained sharp imparted crease and smooth unpuckered seams therein at said locations after repeated washings.

2. A process as defined in claim 1 wherein the impregnation of said fabrics is controlled to an extent that approximately 85% to 100% of the compound by weight is retained in the fabrics.

3. A process as defined in claim 1 wherein said solution is constantly agitated at a temperature ranging between 120° F. and 130° F. and wherein the fabrics containing said solution are dried at a temperature ranging between approximately 200° F. and 220° F.

4. A process for manufacturing garments from cotton fabrics and of any style, size, design and type as defined in claim 1 wherein said aqueous solution of a thermosetting compound comprises urea formaldehyde resin, stearamide with melamine formaldehyde dispersion, a water soluble metallic salt and a wetting agent in approximately 50 gallons of water.

5. A process of manufacturing garments from viscose rayon and of any style, size, design and type, as defined in claim 1, and wherein said aqueous solution comprises approximately 12 gallons of an aqueous composition of a urea formaldehyde resin comprising approximately 50% water and 50% resin, approximately 16 pounds of stearamide with a melamine formaldehyde resin dis-

persion in the proportion by weight of 33 parts of stearamide to 67 parts of melamine formaldehyde resin, approximately 15 pounds of an aqueous solution of magnesium chloride hexahydrate, approximately 2 pounds of a polyvinyl alcohol, approximately one quart of a wetting agent, all in approximately 50 gallons of water.

5 6. A process as defined in claim 1 for manufacturing garments from 100% cotton wherein said thermosetting compound comprises approximately 6 gallons of an aqueous composition comprising approximately 50% water and 50% of a urea formaldehyde resin, approximately 16 pounds of stearamine with melamine formaldehyde resin dispersion in the proportion of 33% steramide and 67% resin, by weight approximately 7½ pounds of 10 magnesium chloride hexahydrate, a wetting agent and water sufficient to bring the solution to 50 gallons.

15 7. A process as defined in claim 6, and including approximately 12 pounds of a polyethylene emulsion in said aqueous solution of a thermosetting compound.

20 References Cited by the Examiner

UNITED STATES PATENTS

|           |         |                      |             |
|-----------|---------|----------------------|-------------|
| 2,846,337 | 8/1958  | Cooke et al. -----   | 38—144 X    |
| 2,876,062 | 3/1959  | Torke -----          | 38—144 X    |
| 2,933,409 | 4/1960  | Binkley -----        | 38—144 X    |
| 2,950,553 | 8/1960  | Hurwitz -----        | 117—139.4 X |
| 2,957,746 | 10/1960 | Buck et al. -----    | 38—144 X    |
| 2,974,432 | 3/1961  | Warnock et al. --    | 117—139.4 X |
| 3,015,584 | 1/1962  | Reinhardt et al. --- | 117—139.4   |
| 3,025,622 | 3/1962  | Hilton -----         | 38—144      |
| 3,051,674 | 8/1962  | Kress -----          | 260—29.4    |
| 3,055,773 | 9/1962  | Mosher -----         | 260—29.4    |
| 3,094,705 | 6/1963  | Reid et al. -----    | 38—144 X    |
| 3,096,524 | 7/1963  | Mizell -----         | 2—243       |

JORDAN FRANKLIN, Primary Examiner.

G. V. LARKIN, Assistant Examiner.

**Dedication**

3,268,915.—*William K. Warnock*, Kentfield, and *Frank G. Hubener*, San Carlos, Calif. PROCESS OF MANUFACTURING PRESS-FREE GARMENT WITH RETAINED CREASES. Patent dated Aug. 30, 1966. Dedication filed May 18, 1970, by the assignee, *Koratron Company, Inc.*

Hereby dedicates the remaining term of said patent to the Public.  
[*Official Gazette August 18, 1970.*]